

## 1

3,003,961

GLYCINE IMIDES IN TURBINE OIL  
 Harry J. Andress, Jr., Pitman, and Paul Y. C. Gee,  
 Woodbury, N.J., assignors to Socony Mobil Oil Company, Inc., a corporation of New York  
 No Drawing. Filed June 10, 1959, Ser. No. 819,234  
 4 Claims. (Cl. 252—33.6)

This invention relates to antirust compositions. It is more particularly concerned with mineral lubricating oils containing certain succinimides and salts thereof.

As is well known to those skilled in the art, the rusting of ferrous metal surfaces has been a common occurrence in the field of lubrication. This has been a serious problem in steam turbine lubrication, particularly during the initial operation of new installations. Rusting is most pronounced at points where the clearance between bearing surfaces is very small, as in the governor mechanism. This is usually caused by water entering the oil supply, as by condensation, and becoming entrained in the oil throughout the circulating system, thereby coming into contact with the ferrous metal surfaces. Manifestly, this constitutes a menace to the operational life of the turbine.

Many materials have been proposed as addition agents to impart antirust properties to lubricating oils. Particularly, in the case of rust protection in the presence of sea water, as in marine turbine lubrication, most compounds used have been materials containing two or more carboxylic acid groups (—COOH). Monocarboxylic acids have generally not been effective in marine service.

It has now been found that antirust properties in the presence of sea water can be imparted to lubricating oil by the addition of certain cyclic imides. It has been discovered that certain alkenyl succinimides and amine salts thereof are effective antirust additives for turbine oils.

Accordingly, it is a broad object of this invention to provide novel rust inhibitors. Another object is to provide lubricating oils that are inhibited against rusting of ferrous metal surfaces in the presence of sea water. A further object is to provide an antirust turbine oil containing succinimide rust inhibitors. A specific object is to provide a turbine oil containing certain alkenyl succinimides and salts thereof. Other objects and advantages of this invention will become apparent to those skilled in the art from the following detailed description.

In general, the present invention provides a mineral lubricating oil containing a small amount, sufficient to prevent rusting of ferrous metal surfaces, of (1) an N-carboxymethyl-alkenyl succinimide containing between about 8 carbon atoms and about 35 carbon atoms in the alkenyl group or (2) the salts of (1) with tertiary-alkyl primary amines having a tertiary carbon atom attached to the nitrogen atom and containing between about 6 carbon atoms and about 30 carbon atoms per tertiary alkyl radical.

The novel addition agents utilizable in this invention are N-carboxymethyl-alkenyl-succinimides and amine salts thereof with tertiary-alkyl primary amines. The succinimides contemplated herein can be prepared by several methods known to the art for making cyclic imides. Most feasibly, they are prepared by reacting an alkenyl succinic acid anhydride or an alkenyl succinic acid with glycine (aminoacetic acid) in equimolar

## 2

amounts and with the elimination of water of condensation. In the case of the anhydride, there will be formed one mole of water per mole of reactant, and with the acid, two moles of water are formed. Accordingly, the condensation will be carried out at temperatures of between about 150° C. and about 250° C., preferably between about 175° C. and about 200° C. The time of reaction will be dependent, of course, upon the reaction temperature employed. Reaction will continue until the required amount of water of condensation has evolved. Generally, the time will vary between about 2 hours and about 6 hours. Shorter reaction times are required if water is removed by azeotropic distillation. Suitable liquids which form azeotropes with water are non-polar solvents, such as benzene, toluene, xylenes, etc.

The alkenyl succinic acid anhydride reactant can have between about 8 and about 35 carbon atoms in the alkenyl radical, and preferably between about 10 and about 14 carbon atoms. Non-limiting examples of the alkenyl succinic acid anhydride reactants are octenyl succinic acid anhydride, diisobutetyl succinic acid anhydride, 2-methylheptenyl succinic acid anhydride, 4-ethylhexenyl succinic acid anhydride, nonenyl succinic acid anhydride, decenyl succinic acid anhydride, undecenyl succinic acid anhydride, dodecenyl succinic acid anhydride, triisobutetyl succinic acid anhydride, tetrapropenyl succinic acid anhydride, tetradecenyl succinic acid anhydride, hexadecenyl succinic acid anhydride, 11-tricosenyl succinic anhydride, and 17-pentatriacontenyl succinic anhydride. As mentioned hereinbefore, the alkenyl succinic acids corresponding to these alkenyl succinic acid anhydrides can be used to prepare the compounds of this invention.

The amine salts of the N-carboxymethyl-alkenyl-succinimides are prepared readily by warming the succinimide with an equimolar amount of tertiary-alkyl primary amine. The addition takes place readily, without the elimination of water, but it is facilitated by heating to temperatures of between about 50° C. and about 100° C.

The amines utilizable in forming the salts of the N-carboxymethyl-alkenyl-succinimides are the tertiary-alkyl, primary, monoamines in which a primary amino (—NH<sub>2</sub>) group is attached to a tertiary carbon atom and which contain between about 6 carbon atoms and about 30 carbon atoms in the tertiary-alkyl radical; and mixtures thereof. These amines all contain the terminal group,



Non-limiting examples of the amine reactants are t-hexyl primary amine, t-octyl primary amine, t-nonyl primary amine, t-decyl primary amine, t-dodecyl primary amine, t-tetradecyl primary amine, t-octadecyl primary amine, t-eicosyl primary amine, t-docosyl primary amine, t-tetraicosyl primary amine, and t-triacontyl primary amine. The amine reactants can be prepared in several ways well known to those skilled in the art. Specific methods of preparing the t-alkyl primary amines are disclosed in the Journal of Organic Chemistry, vol. 20, page 295 et seq. (1955). Mixtures of such amines can be made from a polyolefin fraction (e.g., polypropylene and polybutylene cuts) by first hydrating with sulfuric acid and water to the corresponding alcohol, converting the alcohol to alkyl chloride with dry hydrogen chloride, and

finally condensing the chloride with ammonia, under pressure, to produce a t-alkyl primary amine mixture.

The N-carboxymethyl-alkenyl-succinimides and the amine salts have the structures, respectively:



and



wherein R is an alkenyl group containing between 8 and 35 carbon atoms, preferably between 10 and 14 carbon atoms, and R' is a tertiary-alkyl radical containing between about 6 and about 30 carbon atoms.

The N-carboxymethyl-alkenyl-succinimides and salts contemplated herein are effective to impart antirust properties to mineral lubricating oils, particularly highly refined mineral lubricating oils, such as, steam turbine oils. The amount of succinimide or salt that is added to the lubricating oil will vary between about 0.001 percent and about 10.0 percent, by weight of the oil. In preferred practice, amounts varying between about 0.05 percent and about 1.0 percent, by weight, are used. Other substances can be added to the lubricating oil to impart other properties thereto. For example, there may be added antioxidants, pour point depressants, V.I. improvers, and E.P. agents.

The following specific examples are for the purpose of illustrating the antirust lubricants of this invention and of demonstrating the effectiveness thereof. It is to be understood that this invention is not to be limited to the particular reactants employed, or to the operations and manipulations described therein. Other reactants, as described hereinbefore, can be employed, as those skilled in the art will readily understand.

#### AMIC ACIDS AND SALTS

The salt-forming amine reactant used in the specific working examples is a mixture of pure amines. "Amine A" is a mixture of primary amines having a carbon atom of a tertiary butyl group attached to the amino ( $-\text{NH}_2$ ) group and containing 12 to 15 carbon atoms per amine molecule and averaging 12 carbon atoms per molecule. This mixture contains, by weight, about 85 percent tertiary dodecyl amine, about 10 percent tertiary pentadecyl amine, and relatively small amounts, i.e., less than about 5 percent of amines having less than 12 or more than 15 carbon atoms.

#### Example 1

A mixture of 37.5 grams (0.5 mole) glycine and 150 grams (0.5 mole) tetrapropenyl-succinic anhydride were slowly heated to a temperature of about 200° C. over a period of about 12 hours. Nine grams (0.5 mole) of water were evolved during the course of the reaction.

#### Example 2

A mixture of 37.5 grams (0.5 mole) glycine and 150 grams (0.5 mole) tetrapropenyl succinic anhydride were slowly heated to a temperature of about 200° C. over a period of about 12 hours. The mixture was cooled to about 75° C. and 100 grams (0.5 mole) of amine A was added. The mixture was stirred for about 2 hours at 100° C. to insure complete reaction.

#### Example 3

Two mineral oil blends were prepared. Each blend contained a small amount of one of the additives described in Examples 1 and 2. Two base oils were used.

- 5 Oil X is a highly solvent-refined mineral lubricating oil having 31° API gravity and a Saybolt Universal Viscosity of 150 seconds at 100° F. Oil Y is a highly solvent refined Mid-Continent oil having 29° API gravity and a Saybolt Universal Viscosity of 415 seconds at 100° F. Both are typical steam turbine lubricating oils. These blends were subjected to the ASTM Rust Test D665-44T using synthetic sea water. The composition of each blend and test result are set forth in Table I.

The test method used to distinguish the rusting characteristics of lubricating oil blends was the ASTM test D665-44T for determining "Rust Preventing Characteristics of Steam Turbine Oils in Presence of Water," in which synthetic sea water was used. The synthetic sea water contained 25 grams of sodium chloride, 11 grams of magnesium chloride hexahydrate, 4 grams of sodium sulfate, and 1.2 grams of calcium chloride per liter. In this test a cylindrical polished steel specimen is suspended and soaked in 300 cubic centimeters of the oil under test at 140° F. for thirty minutes. Thirty cubic centimeters of synthetic sea water are added and the mixture is stirred at 1000 r.p.m. After 48 hours, the steel specimen is removed and examined for evidence of rust on the portion of the specimen which hangs in the oil. In order to pass this test, the test specimen must be entirely free 30 of rust.

| Additive of Example | Concn,<br>Wt.<br>Percent | Base<br>Oil | ASTM<br>Rust<br>Test<br>Result |
|---------------------|--------------------------|-------------|--------------------------------|
|                     |                          |             |                                |
| 1                   | none                     | X           | Fail.                          |
| 2                   | 0.10                     | X           | Pass.                          |
|                     | 0.05                     | Y           | Pass.                          |

45 It will be apparent to those skilled in the art that the alkenyl succinimides and amine salts thereof are effective to impart antirust properties to lubricating oils, in the presence of sea water. Thus, the mineral oil compositions are highly effective for severe service, such as, in marine turbine lubrication.

50 Although the present invention has been described with preferred embodiments, it is to be understood that modifications and variations may be resorted to, without departing from the spirit and scope of this invention, as 55 those skilled in the art will readily understand. Such variations and modifications are considered to be within the purview and scope of the appended claims.

What is claimed is:

1. A mineral lubricating oil containing a small amount, sufficient to prevent rusting of ferrous metal surfaces, of at least one compound selected from the group consisting of (1) an N-carboxymethyl-alkenyl-succinimide containing between about 8 carbon atoms and about 35 carbon atoms in the alkenyl group and (2) amine salts of (1) with tertiary-alkyl primary amines having a tertiary carbon atom attached to the nitrogen atom and containing between about 6 carbon atoms and about 30 carbon atoms per tertiary-alkyl radical.
2. The lubricating oil composition defined in claim 1, wherein said mineral lubricating oil is a steam turbine lubricating oil and wherein said compound is present in amounts varying between about 0.001 percent and about 10 percent, by weight of the oil.
3. A steam turbine lubricating oil containing between

about 0.05 percent and about one percent, by weight of the oil, of N-carboxymethyl-tetrapropenyl-succinimide.

4. A steam turbine lubricating oil containing between about 0.05 percent and about one percent, by weight of the oil, of an amine salt of N-carboxymethyl-tetrapropenyl-succinimide, wherein the salt-forming amine is a mixture of tertiary-alkyl primary amines having a tertiary carbon atom attached to the nitrogen atom and containing between 12 and 15 carbon atoms per tertiary-alkyl

radical and having an average of about 12 carbon atoms per molecule.

References Cited in the file of this patent

UNITED STATES PATENTS

2,604,451 Rocchini \_\_\_\_\_ July 22, 1952  
2,790,779 Spivack et al. \_\_\_\_\_ Apr. 30, 1957